

## UNITED STATES PATENT OFFICE.

ANTON AAGAARD, OF EVERETT, WASHINGTON.

## WATERPROOF LEATHER DRESSING AND PRESERVATIVE.

SPECIFICATION forming part of Letters Patent No. 764,971, dated July 12, 1904.  
Application filed January 27, 1904. Serial No. 190,876. (No specimens.)*To all whom it may concern.*

Be it known that I, ANTON AAGAARD, a citizen of the United States, residing at Everett, in the county of Snohomish and State of Washington, have invented certain new and useful Improvements in Waterproof Leather Dressings and Preservatives; and I do hereby declare the following to be a full, clear, and exact description of the invention, such as will enable others skilled in the art to which it appertains to make and use the same.

My invention relates to improvements in waterproof leather dressing and preservative, admirably adapted to preserve and render soft, pliable, and waterproof the leather to which it is applied.

In manufacturing my new composition I use tar made from the roots of pine trees, preferably the so-called "Stockholm" or "Norwegian" tar, dogfish-oil, (*Squalus suckleyi*), and turpentine in the following proportions: five parts pine-root tar, fourteen parts dogfish-oil, one part turpentine. These are mixed well together and boiled, as follows: If the dogfish-oil (*Squalus suckleyi*) has been procured by "trying out" the livers by heat, then the compound need be boiled but from fifteen to twenty-five minutes. If the dogfish-oil is "raw"—that is, oil drawn from the livers without heat—then the whole mixture must be boiled from thirty to forty-five minutes. The duration of the boiling period is material, as if the mixture is boiled for a less time than is required there will not be a thorough mixture of the ingredients, whereas if boiled for too long a period of time the mixture will become hard and brittle and of little value as a leather-dressing, and the exact time of boiling must be determined by the results thereby obtained, as determined by the tests.

The pine-root tar is commonly called "Stockholm" or "Norwegian" tar and differs from the tar procured from the Carolinas in that the Stockholm tar does not contain any granular substance which would tend to injure the leather.

It is desirable to use the turpentine, as there-

by better results are obtained; but the proportion of turpentine may be varied greatly and in some instances entirely omitted without material loss of efficiency.

The oil employed in the present process for making waterproof leather-dressing is obtained from the liver of a fish commonly known as "dogfish," (*Squalus suckleyi*.) I preferably procure the oil from the liver by steam heat while the liver is fresh, the oil thus containing no granulous substances and no harsh fish odor, and by boiling this oil together with the tar above specified the compound becomes very thin, so that when it is applied to leather it is absorbed thereby into the pores, and there remains no greasy matter on the surface of the leather, thereby producing results of material advantage to the leather, such as the softening and preservation thereof.

The mixture when properly boiled and cooled serves as a waterproof preservative dressing for leather which is unexcelled in efficiency. Owing to the nature of the ingredients, when the mixture is applied to the leather the oil will soften the same and the tar, filling the pores of the leather, will render it impervious to moisture.

Having thus fully described my invention, what I claim as new, and desire to secure by Letters Patent, is—

1. A leather-dressing comprising a mixture of dogfish-oil and pine tar.
2. A leather-dressing comprising a mixture of dogfish-oil and pine-root tar.
3. A leather-dressing comprising a mixture of dogfish-oil, pine-root tar and turpentine.
4. A leather-dressing comprising a mixture of dogfish-oil, from five to fourteen parts, pine-root tar, from one to five parts, and turpentine.
5. A leather-dressing comprising a mixture of fourteen parts dogfish-oil, and five parts pine-root tar substantially free from granular material.
6. A leather-dressing comprising a mixture of dogfish-oil and tar.
7. A leather-dressing comprising a mixture of dogfish-oil, turpentine, and tar.

8. A leather-dressing, comprising a mixture of dogfish-oil, turpentine, and another dissolvent.
9. A leather-dressing, comprising a mixture of dogfish-oil, turpentine, and pine tar.
10. A leather-dressing, comprising a mixture of dogfish-oil and a suitable dissolvent.

In testimony whereof I hereunto affix my signature in presence of two witnesses.

ANTON AAGAARD.

Witnesses:

G. WARD KEMP,  
C. C. PHILLIPS.